

# UNITED STATES PATENT OFFICE.

WALTER RÜBEL, OF BERLIN, GERMANY, ASSIGNOR TO RÜBEL BRONZE LIMITED, OF LONDON, ENGLAND.

## ALLOY.

1,076,455.

Specification of Letters Patent. Patented Oct. 21, 1913.

No Drawing.

Application filed June 23, 1913. Serial No. 775,359.

*To all whom it may concern:*

Be it known that I, WALTER RÜBEL, a subject of the Emperor of Germany, residing at Berlin, Germany, have invented a new and useful Alloy, of which the following is a specification.

This invention relates to an improved iron - nickel - aluminium - manganese alloy, which is adapted to be mixed with metals to form other alloys, for example, it may be mixed with copper and aluminium to form a bronze.

According to the invention, iron, nickel, manganese, and aluminium are melted together in proportions corresponding to the multiples of their atomic weights, expressed in the following formula, viz:

$$4(\text{FeNi}) + 8\text{Al} + \text{Mn}.$$

Thus

$$4(55.9 + 58.6) + 8 \times 27.02 + 55$$

gives the following percentage composition: iron 30.67, nickel 32.14, aluminium 29.64, manganese 7.54.

Small variations from the above propor-

tions can be made; for example, an alloy having the following composition has been found to give good results: 31 parts by weight of iron, 32 parts by weight of nickel, 30 parts by weight of aluminium, 30 7.5 parts by weight of manganese.

What I claim is:

1. An alloy consisting of iron, nickel, manganese and aluminium melted together in proportions corresponding to the multiples of their atomic weights expressed in the following formula, viz:

$$4(\text{FeNi}) + 8\text{Al} + \text{Mn}.$$

40

2. An alloy consisting of the following metals melted together in the following proportions by weight, viz:—iron 31 parts, nickel 32 parts, aluminium 30 parts and manganese 7.5 parts.

WALTER RÜBEL.

Witnesses:

ARTHUR ORTH,  
RICHARD JENKEL.